

# United States Patent Office

3,287,268

Patented Nov. 22, 1966

1

3,287,268

CUTTING OIL CONTAINING DEFOAMANT  
Frederick E. Tice, Bayonne, N.J., assignor to Esso Research and Engineering Company, a corporation of Delaware  
No Drawing. Filed Nov. 21, 1963, Ser. No. 325,483  
4 Claims. (Cl. 252—48.4)

The present invention relates to improvements in sulfurized or chlorinated cutting oils and is particularly concerned with the modification of such oils to reduce their foam-forming tendencies.

Cutting oils serve to remove the heat generated during machining of metal and to lubricate the cutting tool against the work and chips. The types of cutting oils employed vary greatly, depending upon the cutting conditions and the metals being cut. For most commonly encountered cutting operations employing various steels and cast iron, the so-called transparent cutting oils which contain sulfur and/or chlorine compounds are widely used and do an excellent job.

Because of the need for a large quantity of cutting oil during the cutting operation, the oil is often sprayed at high pressure into the cutting zone. In addition, in many operations, the chips and turnings which accumulate at the machine are collected and centrifuged to recover the cutting oil which is then returned to the machine. These two factors viz., spraying and centrifuging, as well as other factors associated with a circulating cutting oil system promote the formation of foam. In order to prevent this objectional foam-forming tendency of the cutting oil, a defoaming agent may be employed. In some environments, well-known silicone defoamants are employed. However, in certain instances the use of silicone is prohibited. An example of such an instance is in those operations where the metal being machined is subsequently painted. Here, the presence of silicone, even in minute quantities, cannot be tolerated.

By means of the present invention there is provided a nonsilicone-containing defoamant for sulfurized and/or chlorinated cutting oil. In addition, there are provided an improved cutting oil composition which exhibits anti-foamant properties and a method for reducing the foaming encountered in circulating cutting oil systems.

According to the present invention, it has been surprisingly found that the use of about 0.05 to 0.5 volume percent of an alkenyl succinic acid ester derivative in a cutting oil, hereinafter defined, effectively reduces the tendency of the oil to produce foam and lessens the stability of the foam that is produced.

The alkenyl succinic acid ester derivative employed in the present invention comprises a mixture of an alkenyl succinic acid and an ester formed from that acid, or from a related alkenyl succinic acid containing about 8 to 30 carbon atoms in the alkenyl group, and a glycol of 2 to 4 carbon atoms.

The mixture of acid and ester may be prepared by reacting an alkenyl succinic anhydride with about an equimolar quantity of a glycol at a temperature of about 75 to 400° F., for about 1 to 24 hours, followed by the addition of an additional quantity of the same or a related alkenyl succinic anhydride and about an equimolar quantity of water. This preparation may, if desired, be carried out in a mineral oil diluent.

The preparation of alkenyl succinic anhydrides is well known in the art and simply involves the reaction of maleic anhydride with an olefinic compound, usually in equimolar proportions, though in some cases somewhat of an excess of olefinic material is used. Generally, the reaction involves simple heating, but in other cases catalytic means may be employed. Since relatively pure olefins

2

are difficult to obtain or are often too expensive for commercial use, alkenyl succinic acid anhydrides are ordinarily prepared as mixtures by reacting mixed olefins with maleic anhydride. Such mixtures, as well as relatively pure alkenyl succinic anhydrides, may be employed in this invention. Mixed alkenyl succinic anhydrides wherein the alkenyl group averages 6 to 8, 8 to 10, and 10 to 12 carbon atoms, are commercially available.

Alkenyl succinic anhydrides can also be prepared by reaction of low molecular weight polymers of  $C_2$  to  $C_4$  olefins with maleic anhydride. Thus, a  $C_{12}$  or a  $C_{16}$  alkenyl succinic anhydride can be prepared in this manner from tetrapropylene or from tetraisobutylene, respectively.

10 While the preferred derivative is the hereinafter described mineral oil concentrate containing a mixture of tetrapropenyl succinic acid and the monoester of said acid with propylene glycol, other alkenyl succinic acid derivatives as well as other methods of preparation may be used. (By tetrapropenyl is meant the  $C_{12}$  alkyl group derived from tetrapropylene.) For example, the ester may be prepared by using  $C_2$  to  $C_4$  glycols, such as ethylene glycol, or butylene glycol; the acid may be any alkenyl succinic acid wherein the alkenyl group contains from about 8 to 30 carbon atoms, for example,  $C_8$  from diisobutylene,  $C_9$  from tripropylene,  $C_{15}$  from pentapropylene,  $C_{20}$  to  $C_{24}$  from polyisobutylene of about 300 molecular weight, etc.; the relative proportions of said acid and said ester may vary widely but will usually range from about 40 to 80 volume percent acid and 20 to 60 volume percent ester. In addition, the derivative may be prepared with or without the use of a petroleum diluent. Thus, the amount of diluent may also vary widely, for example, from about 0 to 80 weight percent, preferably from about 30 to 50 weight percent.

20 The derivative may be prepared from two different alkenyl succinic acids, for example, the free acid may be diisobutylene succinic acid and the monoester may be prepared from butylene glycol and tripropylene succinic acid. An ester containing terminal hydroxy groups may be prepared by reacting about equimolar quantities of the alkenyl succinic acid with an alkylene oxide of from 2 to 4 carbon atoms, for example, ethylene oxide, propylene oxide or butylene oxide.

25 The alkenyl succinic acid ester derivative preferred for use comprises 60 weight percent of a mixture of 60 volume percent tetrapropenyl succinic acid, 40 volume percent monoester of tetrapropenyl succinic acid with 1,2-propane diol, and 40 weight percent of a petroleum diluent. 30 This derivative may be prepared by reacting about 0.4 mole of tetrapropenyl succinic anhydride in mineral oil with 0.4 mole of propylene glycol at a temperature of about 75 to 400° F., preferably 180 to 250° F. for about 1 to 24 hours, preferably 3 to 5 hours, followed by the 35 addition of 0.6 mole of tetrapropenyl succinic anhydride and 0.6 mole of water and hydrolysis at about 75 to 300° F., preferably 160 to 200° F.

40 The cutting oils to which the succinic acid derivative may be added in accordance with the present invention are the so-called transparent cutting oils and the black oils. Both oils are characterized by the presence of sulfur and/or chlorine-containing materials which impart extreme pressure properties to the oils. The black oils differ from the transparent oils in that the former contain larger amounts of sulfur and/or chlorine-containing materials than the latter. These oils are well known in the art and the following description of such oils is not intended to limit the present invention in any respect. Such oils include: sulfurized hydrocarbon oils and hydrocarbon oils to which various sulfurized and/or chlorinated materials have been added, such as sulfurized fatty oils, sulfurized solvent extracts of mineral oils, sulfurized

esters, sulfurized olefin polymers, chlorinated waxes, chlorinated aromatics, chlorinated esters, and the like.

Sulfurization is usually accomplished with free sulfur or with sulfur monochloride or with a combination of these agents. The sulfurization of a mineral hydrocarbon oil may be effected, for example, by adding elemental sulfur thereto and heating to 250 to 300° F. or higher. In some instances it is merely necessary to add the sulfur to the mineral oil at a temperature high enough to melt the sulfur, stir the sulfur into the oil, and then cool the mixture.

An animal or vegetable oil such as sperm oil, lard oil, cottonseed oil, peanut oil, or the like, may similarly be sulfurized by adding sulfur thereto, as for example, 6 to 12% sulfur, and heating at a temperature in the range of say 300 to 375° F. for 1 to 3 hours. The sulfurization of the fatty oil may be accomplished in the presence of the fatty oil alone, in which case the sulfurized product is subsequently blended with a mineral lubricating oil, or alternatively, the fatty oil may be sulfurized in the presence of the mineral lubricating oil.

Among the sulfurized materials that may be employed in preparing cutting oils in accordance with the present invention are included: the sulfurized esters of abietic acid described in U.S. Patent 2,217,764, the sulfurized solvent extracts of petroleum fractions described in U.S. Patents 2,222,643 and 2,227,952, the sulfurized olefin polymers described in U.S. Patent 2,246,282, and the sulfurized oils prepared in accordance with U.S. Patents 2,246,282 and 2,467,137. It is to be understood, of course, that the invention is not limited to these particular types of materials.

Chlorination is usually accomplished with elemental chlorine gas. The chlorination of a mineral hydrocarbon may be effected, for example, by contacting the hydrocarbon at 175 to 200° F. with chlorine gas, with or without the aid of a catalyst as desired. The product is subsequently stripped of excess chlorine and hydrogen chloride reaction product and cooled.

Among the chlorinated materials that may be employed in preparing the cutting oils in accordance with the present invention are included: chlorendic acid esters; the sulfurized esters of chlorendic acid described in U.S. Patent 2,969,326; chlorinated aromatics, for example, chlorinated biphenyl; chlorinated wax; chlorinated naphthalenes; and the like.

In general, the cutting oils will contain about 0.1 to 5.0 weight percent sulfur and/or about 0.05 to 5.0 weight percent chlorine, preferably about 0.4 to 0.8 weight percent sulfur and 0.05 to 0.15 weight percent chlorine.

Although a wide range of lubricating oils may be employed as base stocks for these cutting oils, in general the base oil will comprise an oil having a viscosity at 100° F. in the range of from about 90 to 500 Saybolt seconds, an API gravity of from about 23° to about 33°, and a flash point above about 300° F. Preferably, a light coastal petroleum oil or naphthenic petroleum oil having a viscosity at 100° F. from about 100 to about 300 SUS is used.

The following examples serve to illustrate the manner in which the invention may be practiced.

#### Example 1

0.4 mole of tetrapropenyl succinic anhydride and 0.4 mole of propylene glycol are reacted in a mineral oil diluent at a temperature of about 210 to 215° F. for about 4 hours. 0.6 mole of tetrapropenyl succinic anhydride and 0.6 mole of water are then added to the mixture and the anhydride is hydrolyzed at about 180° F. The resulting mixture consists of 60 weight percent of the reaction product and 40 weight percent mineral oil diluent.

#### Example 2

In order to demonstrate the defoamant properties of the additive of Example 1, two cutting oils were prepared

and tested. Cutting oil A was a commercially available sulfur and chlorine-containing oil. This oil (A) consisted of:

|   |                              | Weight percent |
|---|------------------------------|----------------|
| 5 | Base oil <sup>1</sup>        | 98.1           |
|   | Anglamol 31 <sup>2</sup>     | 1.0            |
|   | Sulchlor 1717-M <sup>3</sup> | 0.9            |

<sup>1</sup> Mineral lubricating oil derived from naphthenic distillate having a viscosity of 150 SSU at 100° F.

<sup>2</sup> Lubrizol Corp. additive which contains as active ingredients 42-46% S and a maximum of 0.2 wt. percent Cl.

<sup>3</sup> Carlyle Chemical Works, Inc. additive which contains as active ingredients a minimum of 9.0 wt. percent S and a minimum of 9.0 wt. percent Cl.

Cutting oil B consisted of cutting oil A to which had been added 0.3 volume percent of the additive of Example 1.

Cutting oils A and B were tested for foaming characteristics using the ASTM-D892 Foam Test and for interfacial tension using the ASTM-D971-50 Interfacial Tension Test. The results are shown in Table I.

TABLE I

| Cutting Oil | ASTM-D971-50<br>I.F.T. at<br>25° C. | ASTM-D892         |                    |                |
|-------------|-------------------------------------|-------------------|--------------------|----------------|
|             |                                     | Tendency<br>(cc.) | Stability<br>(cc.) | Time<br>(Min.) |
| A-----      | 21.9                                | 510               | 40                 | 10             |
| B-----      | 11.0                                | 90                | 0                  | 3              |

These results show that cutting oil B, containing a defoamant of the present invention, has a reduced tendency to produce foam and further the small amount of foam that is produced is unstable.

#### Example 3

0.2 mole of diisobutetyl succinic anhydride and 0.2 mole of ethylene glycol are reacted at a temperature of 220° F., for about 5 hours. 0.8 mole of diisobutetyl succinic anhydride and 0.8 mole of water are then added to the mixture and hydrolyzed at about 220° F. for about 2 hours.

#### Example 4

A sulfurized cutting oil was prepared by dissolving at about 250° F., with stirring, about 1 weight percent of elemental sulfur in a naphthenic oil having a viscosity of about 145 SUS at 100° F. and then blending 92.5% of the sulfurized naphthenic oil with 7.5% of mixed fatty oils that had been treated with sulfur monochloride to a content of about 8% sulfur and 8% chlorine. To this cutting oil, 0.15 volume percent of the product prepared in Example III can be added.

It is recognized that many modifications of the instant disclosure may be made without departing from the spirit of the invention as defined by the appended claims. Further, it is not intended that the examples shown limit the invention in any respect.

What is claimed is:

1. An improved cutting oil having a reduced tendency to form foam which comprises a major proportion of a lubricating oil having a viscosity at 100° F. within the range between about 90 to 500 SUS, about 0.05 to 10 weight percent of an oil-soluble compound selected from the group consisting of sulfurized compounds and chlorinated compounds, and about 0.05 to 0.5 volume percent of a mixture of (a) an alkenyl succinic acid and (b) the monoester of an alkenyl succinic acid and a glycol containing 2 to 4 carbon atoms; wherein said alkenyl groups in said acid and in said ester each contain about 8 to 30 carbon atoms.
2. An oil according to claim 1 wherein said mixture comprises about 60 volume percent of tetrapropenyl succinic acid and about 40 volume percent of the monoester of tetrapropenyl succinic acid with propylene glycol.
3. An improved cutting oil having a reduced tendency

to form foam which comprises a major proportion of a lubricating oil having a viscosity at 100° F. within the range between about 90 to 500 SUS, a minor amount, sufficient to improve the extreme pressure properties of said cutting oil of an oil-soluble compound selected from the group consisting of sulfurized materials and chlorinated materials, and about 0.05 to 0.5 volume percent of an alkenyl succinic acid derivative, said derivative consisting of (a) about 40 to 80 volume percent alkenyl succinic acid, wherein the alkenyl group contains from about 8 to 30 carbon atoms, and (b) 20 to 60 volume percent of the monoester of a glycol which contains from 2 to 4 carbon atoms and an alkenyl succinic acid wherein the alkenyl group contains from about 8 to 30 carbon atoms.

4. An oil as defined by claim 3 wherein the alkenyl

groups of (a) and (b) are both C<sub>12</sub> groups derived from tetrapropylene and said glycol is propylene glycol.

References Cited by the Examiner

UNITED STATES PATENTS

|    |           |         |                      |          |
|----|-----------|---------|----------------------|----------|
| 5  | 2,208,161 | 7/1940  | Prutton et al. ----- | 252—48.8 |
|    | 2,318,629 | 5/1943  | Prutton -----        | 252—48.8 |
|    | 2,394,909 | 2/1946  | Gleason -----        | 260—48.5 |
|    | 2,748,086 | 5/1956  | Monson -----         | 252—358  |
| 10 | 3,004,923 | 10/1961 | Jurisch -----        | 252—358  |

FOREIGN PATENTS

896,376 5/1962 Great Britain.

DANIEL E. WYMAN, Primary Examiner.

15 L. G. XIARHOS, Assistant Examiner.